

## UNITED STATES PATENT OFFICE

2,131,764

## ART OF NITRATING CELLULOSE BY PRE-TREATMENT OF THE CELLULOSE

Fred Bacon Stieg, New York, N. Y., assignor to Rayonier Incorporated, San Francisco, Calif., a corporation of Delaware

No Drawing. Application March 28, 1935,  
Serial No. 13,481

5 Claims. (Cl. 260—146)

My invention relates to the art of nitrating cellulose. More particularly, my invention relates to the nitration of a cellulose especially prepared to facilitate nitration, irrespective of nature, source, physical condition or reactivity of the cellulose, mixture of celluloses or cellulosic material so nitrated, or the nature, physical condition and properties of the nitrated cellulose produced as the result of the application of my invention.

5 The primary object of my invention is to facilitate the converting of cellulose into nitrocellulose which, I have found, may be achieved in a very advantageous manner by pretreating the cellulose with certain chemicals and then proceeding with the usual nitrating process. By treating the cellulose according to my invention, I have discovered that the cellulose nitrates more rapidly and accordingly, the time of nitration may be thereby reduced and a more satisfactory nitration insured. Also I have discovered that the chemicals used in the pretreatment of the cellulose, according to my invention, have no practical interfering effect with the nitration process. That is, the pretreatment according to 15 my invention does not substantially interfere with the desirable properties of the finished product, such as the properties of solubility, viscosity, stability, thermoplasticity or film-forming capacity.

20 For purposes of definiteness of description and illustration, I will set forth my invention as applied to cellulose derived from wood, and especially such cellulose when provided in its manufacture in sheet form, but it is to be expressly understood that it is not to be limited to any such specific application, but extends to all applications where like problems obtain in whole or in part.

25 At the present time, bulk cotton linters derived from cotton are commonly used for producing nitrocellulose, and the period for nitration of such cellulose ordinarily required is about thirty minutes.

30 In the common production of wood pulp for various purposes, it is common practice to provide it in sheet form dried on a paper machine. The sheet form of wood pulp is almost universally sold in unbeaten condition, varying in thickness, weight and porosity. When wood pulp is produced in this way the sheet is relatively thick and dense as compared with the physical forms of cellulose commonly nitrated at the present time. Thus, in the nitration of wood pulp, as it is commonly produced in pulp mills, difficulties are 35 encountered, due to the slow penetration of the

nitrating acid into the sheet and/or the slow rate of nitration and/or non-uniform nitration.

40 Due to these difficulties, little progress has been made in nitrating wood pulp in the physical form of pulp sheets as manufactured in a pulp mill, except where nitrating acid solutions, containing an unusually high ratio of nitrating components, are used—a process which is considerably more expensive.

45 By experimentation, I have found that it is possible to nitrate the above described sheets of wood pulp with nitrating acid solutions of conventional nitric acid content by immersing the wood pulp in the nitrating acid for a relatively long period of time. In these experiments I cut the sheets into small pieces, as herein described, i. e., one-fourth inch by one-fourth inch squares, for convenience in treating with the said nitrating acid solutions. While such period of nitration varies, depending on the thickness and density of the sheet, I have found that a period of time, varying from one and one-half hours to six hours, is required to obtain proper nitration with such pulp sheets.

50 When referring to the time of nitration, I refer to the time period during which the cellulose is in direct contact with the nitrating acid solution.

55 Thus, a serious objection obtains to the nitration of pulp in sheet form, due to the length of the period of nitration required. In addition, there is an uncertainty as to the completeness and degree of nitration obtained. Due to the lack of uniformity of density, porosity and thickness of the sheet, precise control of the nitrating process is exceedingly difficult. Thus, in the nitration of wood pulp as commonly produced in pulp mills at the present time, difficulties are encountered due to the relatively slow penetrating of the nitrating mixture into the sheet, and the irregular and unsatisfactory nitration of the same, in comparison to the nitration of cotton, which is usually in the flock form, and hence almost immediately receptive to the nitrating mixture. Such uniformity is important and the same is provided by my invention, whereby a nitrocellulose product results which is applicable for forming lacquers, artificial leathers, celluloids, films, filaments, explosives and other commercial applications. Furthermore, existing present factories for manufacturing nitro-cellulose have their apparatus or equipment as well as number and capacity of units, designed and arranged to permit a period of nitration of about thirty minutes. It is, therefore, highly desirable that any process to manufacture nitrocellulose from wood pulp, shall use

substantially the same apparatus as is already now installed and employed for the manufacture of nitrocellulose from said cotton linters. Obviously, it is important that the production capacity of existing nitrating installations should not be reduced.

When applying my invention to the nitration of cellulose from cotton or cellulose from wood the machinery and apparatus for the nitrations will be substantially the same as that now installed and employed for the nitration of bulk cotton linters. That is, when operating according to my invention for the nitration of cellulose as applied to the utilization of apparatus and synchronization of units for the various steps involved from the original cellulose to the finished nitrocellulose, it will be found that the apparatus required is substantially the same and of the same capacity per individual step in the process, as that which now prevails in the nitration and purification of nitrated esters, wherein cotton linters is the initial form of cellulose. Primarily I have in mind the most common machinery and apparatus assembly known as the "mechanical dipper" assembly, but it is to be understood that my invention is to apply to all other machinery and apparatus, intermittent or continuous, capable of producing nitrocellulose. The "displacement process" and "pot method" machinery and apparatus are examples of other installations for batch operation. It is to be expressly understood that, due to the effect which this preliminary treatment has on increasing facility of nitration and diminishing the period of penetration of nitrating mixture in and through the impregnated cellulose, it is both possible and practicable to utilize the cellulose impregnated according to this invention in a continuous manner in sheet form, or otherwise, and in a continuous nitrating apparatus.

Sulphite wood pulp and sulphite wood pulp which has been refined to a higher alpha cellulose content may be advantageously used in the practice of my invention. Ordinarily such pulps are produced in a bleached unbeaten form of high whiteness. For convenience in processing in the present nitrating equipment previously described, it is obviously desirable that the wood pulp sheet should be cut up into small pieces, as such form permits handling in the standard equipment with greater ease. These pieces may be small squares, rectangles, or any other shape which may be conveniently produced and processed. I have found squares measuring one-fourth inch by one-fourth inch to function satisfactorily.

Briefly and in general, my invention may be described as follows: I take cellulose preferably in sheet form, and impregnate it with a water solution of an inorganic compound or at least bring each particle of cellulose into intimate association with such inorganic compound. Then, the aqueous portion is removed from said cellulose material, as by drying, until the impregnated cellulose material has a low moisture content, preferably lower than 2% of water on the basis of "bone dry" condition. After this operation the sheet may be cut up into small pieces and nitrated according to standard methods. I have discovered that certain inorganic compounds only and certain classes of inorganic compounds will produce the desirable results of this invention and otherwise meet the exacting requirements for proper nitration.

I have found that inorganic water soluble compounds of the element boron, such as acids of boron, comprising meta boric acid, ortho boric acid, pyro boric acid and the anhydride of these acids, also salts of such boron acids, sodium perborate, alkali metal salts of boron acids, water soluble alkaline earth metal salts of boron acids, and/or salts of boron acids treated with sufficient mineral acid, such as sulphuric acid, to liberate the boron acid, are preeminently efficient. I have discovered that similar water soluble alkali metal salts of the acids of the elements arsenic, aluminum, manganese and chromium also exert a similar, although somewhat lesser effect in reducing the time of nitration. However, these inorganic compounds are less desirable than the boron compounds previously described, because it is more difficult to eliminate these inorganic compounds from the nitrocellulose during stabilization. I have found no tendency for boron impregnating compounds to remain present in the nitrocellulose after nitration and stabilization as commonly practiced.

The following tabulated experiments show clearly the effect of previously impregnating the sheets with a water solution of an inorganic compound, drying the sheets and then nitrating same.

Experiments 1 to 10, inclusive, show that a wide range of nitrating acid compositions can be used to produce a nitrocellulose of any desired nitrogen content or a range of nitrogen contents from the lowest to the highest, found to be advantageous in the art. The time of nitration in each experiment was thirty minutes. Sulphite wood pulp in sheet form refined to an alpha cellulose content of about 95 to 96%, and having a high white color was used in these experiments. This pulp was cut into one-quarter inch squares. It had an original basis weight of two hundred eight pounds and a thickness of .031 inch. The basis weight refers to the weight in pounds of four hundred eighty (480) sheets twenty four inches by thirty six inches, which is the weight of four hundred fourteen thousand seven hundred twenty (414,720) square inches of pulp sheet. This pulp was uniformly impregnated with a water solution of boric acid and then dried to about 1% water content. At this point the sheet was found to contain close to 5% of boric acid based on the air dry weight of the pulp. The method of impregnating was by spraying.

| Nitration experiment number | Sulphuric acid content of nitrating acid | Nitric acid content of nitrating acid | Water content of nitrating acid | Yield of nitrocellulose | Nitrogen analysis of nitrocellulose | Percent |
|-----------------------------|------------------------------------------|---------------------------------------|---------------------------------|-------------------------|-------------------------------------|---------|
|                             | Percent                                  | Percent                               | Percent                         | Percent                 | Percent                             |         |
| 1                           | 51.00                                    | 30.00                                 | 19.00                           | 143.2                   | 10.83                               | 60      |
| 2                           | 52.50                                    | 30.00                                 | 17.50                           | 151.0                   | 11.39                               |         |
| 3                           | 54.00                                    | 30.00                                 | 16.00                           | 159.5                   | 11.96                               |         |
| 4                           | 52.50                                    | 31.40                                 | 16.10                           | 160.0                   | 11.96                               |         |
| 5                           | 51.37                                    | 33.22                                 | 15.41                           | 163.2                   | 12.02                               |         |
| 6                           | 47.20                                    | 38.33                                 | 14.47                           | 164.4                   | 12.26                               |         |
| 7                           | 52.50                                    | 32.80                                 | 14.70                           | 164.6                   | 12.42                               |         |
| 8                           | 21.35                                    | 70.00                                 | 8.65                            | 166.1                   | 12.44                               | 65      |
| 9                           | 39.59                                    | 47.65                                 | 12.76                           | 166.5                   | 12.49                               |         |
| 10                          | 52.50                                    | 34.20                                 | 13.30                           | 169.5                   | 12.83                               |         |

In addition, my Experiments 11 and 12 show that, when practicing my invention, the temperature of the nitrating acid solution can be varied as is the practice when commercially producing nitrocellulose. The time of nitration was thirty minutes. The cellulose was the same as that used in Experiments 1 to 10, inclusive, and

was impregnated with 5% of boric acid in the same way.

| Nitration experiment number | Sulphuric acid content of nitrating acid | Nitric acid content of nitrating acid | Water content of nitrating acid | Temperature of nitration | Yield of nitro-cellulose | Nitrogen analysis of nitro-cellulose |
|-----------------------------|------------------------------------------|---------------------------------------|---------------------------------|--------------------------|--------------------------|--------------------------------------|
|                             | Percent                                  | Percent                               | Percent                         | °C.                      | Percent                  | Percent                              |
| 10 11.....                  | 50.00                                    | 34.00                                 | 16.00                           | 35                       | 161.2                    | 12.01                                |
| 10 12.....                  | 50.00                                    | 34.00                                 | 16.00                           | 45                       | 156.2                    | 12.13                                |

Further experiments, 13 to 18 inclusive, show the progressive rate of nitration when using this same impregnated pulp. In these experiments the nitrating acid solution had the following composition: sulphuric acid 50.00%, nitric acid 34.00%, and diluent 16.00%. The time of nitration was thirty minutes.

| Nitration experiment number | Time of nitration | Yield of nitro-cellulose | Nitrogen analysis of nitro-cellulose |
|-----------------------------|-------------------|--------------------------|--------------------------------------|
| 13.....                     | Minutes 5         | Percent 153.4            | Percent 10.95                        |
| 14.....                     | 10                | 156.3                    | 11.48                                |
| 15.....                     | 15                | 158.1                    | 11.66                                |
| 16.....                     | 20                | 159.8                    | 11.86                                |
| 17.....                     | 25                | 160.1                    | 11.98                                |
| 18.....                     | 30                | 161.2                    | 12.01                                |

Experiments, 19 to 29 inclusive, show the effect of using other impregnating materials and mixtures of impregnating materials. In all instances the nitrating acid compositions were: sulphuric acid 50%, nitric acid 34.00% and diluent 16.00%. The time of nitration was thirty minutes.

| Nitration experiment number |                                                                 | Yield of nitro-cellulose | Nitrogen analysis of nitro-cellulose |
|-----------------------------|-----------------------------------------------------------------|--------------------------|--------------------------------------|
| 19.....                     | Sulphite pulp with 5% boric acid.                               | Percent 161.2            | Percent 12.01                        |
| 20.....                     | Sulphite pulp with 5% borax previously treated with $H_2SO_4$ . | 157.3                    | 11.84                                |
| 21.....                     | Sulphite pulp with 5% boric acid and 1% sodium perborate.       | 161.1                    | 12.01                                |
| 22.....                     | Sulphite pulp with 4% borax and 1% boric acid.                  | 158.3                    | 11.85                                |
| 23.....                     | Sulphite pulp with 5% boric acid and 1% potassium permanganate. | 158.5                    | 12.00                                |
| 24.....                     | Sulphite pulp with 5% arsenious acid.                           | 153.3                    | 11.90                                |
| 25.....                     | Sulphite pulp with 5% arsenic acid.                             | 151.4                    | 11.49                                |
| 26.....                     | Sulphite pulp with 5% sodium aluminate.                         | 150.5                    | 11.76                                |
| 27.....                     | Sulphite pulp with 5% potassium permanganate.                   | 149.3                    | 11.76                                |
| 28.....                     | Sulphite pulp with 5% potassium dichromate.                     | 134.2                    |                                      |
| 29.....                     | Sulphate pulp with 5% boric acid.                               | 156.5                    | 11.89                                |

60 In Experiment #30 bulk cotton (cotton linters) was impregnated with 5% boric acid and nitrated for only twenty minutes with the nitrating acid composition: sulphuric acid 60.00%, nitric acid 22.50% and diluent 17.50%. The yield was 165.9% and the nitrogen content was 12.01%.

In all of the above recorded 30 experiments, it was found that the resulting nitrocellulose was properly nitrated as evidenced by the usual tests applied, including a high clarity of the dissolved nitrocellulose, and freedom of the same from insoluble fibers.

Nitrocellulose yields mentioned above are yields calculated on a basis of the impregnated cellulose nitrated less the impregnating material

used. I prefer to use a pulp refined to a higher alpha cellulose content. The term "refined to a higher alpha cellulose content" has a definite meaning in the art namely: Ordinarily wood sulphite pulp is of 88% to 89% alpha cellulose content. This is refined by processes well known in the art so that a product may be provided having an alpha cellulose content as desired up to 98 or 99%.

The success of my invention is dependent upon the impregnation of the cellulose with materials having the effect of facilitating the nitration reaction. From extended experiments I have discovered that the agents and classes of agents herein named have the effect of causing a more rapid and thorough wetting of the cellulose with the nitrating acid solution. I have employed the cellulose prepared for nitration, which was used in Experiments 1 to 10 inclusive, and immersed it in the nitrating acid solution and have observed that the pulp impregnated with boric acid became thoroughly wet and penetrated by the said solution in less than one minute, whereas the same pulp not impregnated with boric acid required more than thirty minutes to become thoroughly wet. This does not mean that the nitration processes were completed in these times, in either case. In other words, these experiments indicate beyond all question the great aid that the previous impregnation is to the penetration of the nitrating solution. That is, the results as to time do not mean that the nitration processes were initiated and completed within the stated periods, but are a comparative index of the degree and speed of penetration of nitrating mixture as ordinarily would be the case using wood pulp sheets, in contradistinction to the employment of the same or a similar wood pulp sheet previously treated with boric acid according to my invention. One conversant with the art to which this invention appertains, will appreciate that with speed of penetration comes increased ease of nitration and high stability and other desirable features of the finished nitrocellulose, other factors being equal. This augmentation of acid penetration constitutes an unlooked for and highly important discovery, for by its employment in the art of cellulose nitration, a greater productive capacity is possible with a given unit equipment and a more satisfactory and hence more acceptable nitrocellulose to the arts is possible. Furthermore, with increase of speed of initial nitrating acid penetration comes a more desirable nitration.

Whatever may be the theoretical explanation, it positively remains that the presence of the impregnating compound in the cellulose, and more particularly the compounds of boron, most certainly facilitates nitration by reducing the time of nitration, and that the impregnating compound does not objectionably interfere with the nitrating process or contaminate the finished product. The presence of the impregnating material as disclosed herein enables cellulose thus impregnated to be transformed under normal factory conditions into a highly acceptable nitrocellulose. And it has also been conclusively demonstrated, that the use of the compounds as herein specified, for the purposes disclosed, does not disadvantageously affect the desirable physical properties of the nitrocellulose thus produced. Such pretreatment of the cellulose also provides a product of nitrocellulose superior to that which would result if the same process were carried on without the step of impregnating the cellulose.

prior to nitration. The terms "treating", "pre-treatment" and "impregnation" are used herein broadly to include incorporating with, disseminate therein or otherwise bring into intimate association the compounds herein set forth and 5 cellulose material.

In my experiments, to demonstrate the advantageous effects of certain water soluble impregnating agents for cellulose, I used acids of boron, 10 salts of acids of boron, and salts of acids of boron treated with sulphuric acid, also acids of arsenic, aluminates, permanganates, chromates and mixtures comprising two or more of these chemicals. 15 Of the agents used, those containing the chemical element boron gave the most satisfactory results. I prefer to use ortho boric acid, or meta boric acid or pyro boric acid, or the anhydride of these acids, or the water soluble alkali metal salts of the boric acids previously mentioned, or the water 20 soluble alkaline earth metal salts of the boric acids, whose sulphates are also water soluble.

My experiments show that the amount of these 25 impregnating agents in the pulp have the effect of regulating the time of nitration. In order to bring the time of satisfactory nitration to about thirty minutes, certain amounts of impregnating agent on the weight of the cellulose after drying are required, depending on the thickness and 30 density of the sheet. In Experiments 19 and 20, for example, five percent of boric acid was found to give proper nitration in thirty minutes. In general, amounts from 2-5% have a desirable practical effect. That is, as a generality, amounts of impregnating material of two to five percent 35 by weight, based upon the air dry weight of the cellulose to be nitrated induces the effect desired. This is especially true wherein such boron compounds as an acid of boron or a salt of the same is employed. Amounts above five percent of a 40 boric acid as well as other impregnating agents, were found to give no additional benefit. Since the impregnating agents, especially compounds of boron, are soluble in the nitrating acid solution, a calculated amount of the agent was added to the nitrating acid solution in conducting experiments 45 in order that the nitrating acid would contain an amount of the inorganic impregnating agent equivalent to the amount which would accumulate in the nitrating acid in regular commercial practice, where the nitrating acid is constantly strengthened and then reused. However, 50 the presence of the agent in the nitrating acid solution appears to have no objectionable effect.

In nitration procedures I prefer compounds of 55 the chemical element boron as impregnating materials for the cellulose. Of these I prefer the acids of boron. When impregnating the cellulose, whether by spraying, immersion or by any other means whatsoever, I desire that, subsequent to the removal of water by drying, the 60 inorganic compounds be substantially uniformly distributed throughout the cellulosic material. I prefer to nitrate the thinnest practical sheet of pulp that can be economically made on a paper machine. I have found that such whole 65 sheet or sheets of any convenient size respond as readily to nitration as do the smaller, one-quarter of an inch squares. I prefer nitrating acid compositions, depending upon the percentage of nitrogen desired in the nitro-cellulose, to have 70 the highest practical sulphuric acid content and

the lowest practical nitric acid content. The temperature of the nitrating bath may be varied within the usual commercial limits without affecting the value or operativeness of my invention. In other words, my process in nowise interferes with the manufacturing routine or practice commonly obtaining, but rather conforms to or fits in with said practice. Furthermore, attention is especially called to the fact that the 10 impregnating chemicals of the pretreatment process constituting my invention, do not interfere or affect practically the usual procedure for controlling the nitrogen content or other properties of the nitrocellulose. It is to be understood that my invention is not to be limited to any specific 15 weight or thickness of pulp or to any specific nitrating acid compositions or temperatures of nitrating acid compositions, or to any definite porosity or nitrating acid receptivity. I have varied the thickness and porosity of the pulp 20 sheet within comparatively wide limits, and have found my invention equally applicable thereto.

The size or configuration of the individual pieces of wood pulp to be nitrated is not important. My invention applies as well to the 25 nitration of wood cellulose or other forms of cellulose in rolls of indeterminate lengths, or lengths between the same pieces of small size.

I claim:

1. The process of nitrating substantially un-beaten sheet sulphite cellulose, refined to a higher alpha cellulose content, comprising subjecting such cellulose to impregnation with a water solution consisting essentially of a boron compound; 30 drying the cellulose; and subsequently subjecting such cellulose to a nitrating acid solution.

2. The process of nitrating substantially un-beaten sheet sulphite cellulose, refined to a higher alpha cellulose content, comprising subjecting such cellulose to impregnation with a water solution consisting essentially of a boron compound; 40 drying the cellulose; cutting such sheets into relatively small pieces; and subsequently subjecting such cellulose to a nitrating acid solution.

3. The process of nitrating sheet sulphite wood 45 pulp, refined to a higher alpha cellulose content, comprising subjecting said cellulose to impregnation with a solution consisting essentially of a boron compound to provide said sheet with about 5% of said compound (5% by weight of 50 impregnating agent on the weight of the cellulose after drying); drying the cellulose to a low water content; cutting said sheets into relatively small pieces; and subjecting such cellulose to a nitrating acid solution.

4. The process of nitrating cellulose comprising 55 treating cellulose with a cellulose nitration solution wetting facilitating agent consisting essentially of a boron compound, reducing the moisture content of such treated cellulose, and then subjecting the cellulose to the nitrating acid 60 solution.

5. The process of nitrating cellulose comprising 65 treating wood sulphite cellulose in sheet form with a cellulose nitration solution wetting facilitating agent consisting essentially of a boron compound, reducing the moisture content of such treated cellulose, subdividing said sheets into relatively small segments, and then subjecting 70 the cellulose to the nitrating acid solution.

FRED BACON STIEG. 70